

# UNITED STATES PATENT OFFICE.

JAMES R. ROSE, OF EDGEWORTH, PENNSYLVANIA, AND JOHN HARRIS, OF LAKEWOOD,  
OHIO, ASSIGNORS TO CARBO-OXYGEN COMPANY, OF PITTSBURGH, PENNSYLVANIA,  
A CORPORATION OF DELAWARE.

## GASEOUS FUEL.

1,404,229.

Specification of Letters Patent. Patented Jan. 24, 1922.

No Drawing.

Application filed December 26, 1919. Serial No. 347,456.

To all whom it may concern:

Be it known that we, (1) JAMES R. ROSE,  
(2) JOHN HARRIS, citizens of the United  
States, residing at (1) Edgeworth, (2) Lake-  
wood, in the county of (1) Allegheny, (2)  
Cuyahoga, and State of (1) Pennsylvania,  
(2) Ohio, have invented a certain new and  
useful Improvement in Gaseous Fuel, of  
which the following is a full, clear, and  
exact description.

This invention relates to gaseous fuel,  
and more particularly to a fuel which is par-  
ticularly useful for the purpose of cutting  
metals with great rapidity, where extreme  
15 cleanliness of cutting is not essential. A use  
for which our gas is particularly well suited  
is for cutting scrap iron.

It has been proposed heretofore to mix  
with hydrogen, gases such as illuminating  
20 gas and carbon monoxide, for the purpose  
of imparting visibility to the cone within  
the flame produced by the burning of the  
hydrogen and for certain kinds of cutting  
and welding. As pointed out hereinbefore,  
25 it is the purpose of this invention to produce  
a gas which will enable the cutting opera-  
tion to be performed with greater rapidity  
than can be realized by the aforesaid mix-  
tures. For this purpose we form a mixture  
30 of methane and ethylene with hydrogen in  
the proportions of from  $2\frac{1}{2}\%$  to  $12\frac{1}{2}\%$  by  
volume each of such methane and ethylene  
to the hydrogen constituents. This gas has  
a relatively high carbon content which ma-  
35 terially increases the flame volume and  
heat units over those obtainable by the  
combustion in a blow-pipe of hydrogen  
alone with oxygen, and also produces in the  
flame a visible or luminous cone which en-  
ables the proportions of the gases to be  
40 conveniently adjusted and the flame to be  
applied efficiently to the work.

The carbon content of our gaseous mix-  
ture is lower than that required for operat-

ing on heavy masses of metal and for cut-  
ting cast iron and steel, and corroded, dirty  
and slaggy iron and steel—in which opera-  
tions a large flame volume and high units  
are essential. However, our gaseous mix-  
ture is capable of cutting with much greater  
50 rapidity than can gases having such high  
carbon content.

According to Richards on Metallurgical  
Calculations, published in 1908, the flame  
temperature produced by the combustion of  
the aforesaid gases will be over  $3200^{\circ}$  C.,  
and the variations in the percentages of the  
said gases will cause the following variations  
in the net B. T. U. per cubic foot of mix-  
ture and in the cubic feet of oxygen re-  
quired for the combustion of a cubic foot of  
such mixture:

No. 1 mixture, 95% H. with  $2\frac{1}{2}\%$  each of  
ethylene and methane; net B. T. U.'s 344;  
cu. ft. of oxygen, .600.

No. 2 mixture, 75% H. with  $12\frac{1}{2}\%$  each of  
ethylene and methane; net B. T. U.'s 544;  
cu. ft. of oxygen, 1.000.

Having thus described our invention,  
what we claim is:—

1. A gas for cutting, welding and heating  
purposes consisting of a mixture of methane  
and ethylene with hydrogen in the propor-  
tions of from  $2\frac{1}{2}\%$  to  $12\frac{1}{2}\%$  by volume each  
of methane and ethylene to hydrogen.

2. A gas for cutting, welding and heating  
purposes consisting of a mixture of methane  
and ethylene with hydrogen in proportions  
not substantially less than 5% by volume  
of such combined gases to the hydrogen and  
not materially more than 25% of such com-  
bined gases to the hydrogen, the methane and  
ethylene being present in the proportions of  
at least  $2\frac{1}{2}\%$  each in such mixture.

In testimony whereof, we hereunto affix  
our signatures.

JAMES R. ROSE,  
JOHN HARRIS.